

Aug. 9, 1949.

J. J. GREBE ET AL

2,478,479

CORED MAGNESIUM ANODE IN GALVANIC PROTECTION

Filed Feb. 3, 1947



Fig. 1



Fig. 2

INVENTORS.  
John J. Grebe  
Harold A. Robinson  
BY

Griswold & Burdick  
ATTORNEYS

## UNITED STATES PATENT OFFICE

2,478,479

## CORED MAGNESIUM ANODE IN GALVANIC PROTECTION

John J. Grebe, Oak Ridge, Tenn., and Harold A. Robinson, Midland, Mich., assignors to The Dow Chemical Company, Midland, Mich., a corporation of Delaware

Application February 3, 1947, Serial No. 725,982

4 Claims. (Cl. 204—197)

1

This invention relates to systems for the galvanic protection of corrodible metal structures using improved cored magnesium anodes.

In the galvanic protection of pipelines and other underground steel structures, consumable electrodes of a metal anodic to the steel are buried in the earth near the structure and are connected to it by electrical conductors. The resulting flow of current maintains the structure cathodic with respect to the soil and greatly minimizes its corrosion.

The consumable anodes heretofore used have conventionally consisted of a body of a highly electronegative metal, such as magnesium or zinc, cast about a steel core. The core is required in order to maintain structural unity of the anode as the active metal is consumed. With magnesium anodes, however, steel cores are somewhat disadvantageous in that, as soon as any part of the steel is exposed by consumption of the magnesium, a strong local electrolytic couple is set up between the core and the outer metal which, under unfavorable conditions, results in appreciable consumption of the magnesium.

It is therefore the principal object of the present invention to provide a galvanic protection system using an improved cored magnesium anode which is not subject to the disadvantages mentioned.

The improved consumable anode used in the present invention consists essentially of a core of an alloy containing from about 1 to about 92 percent by weight of magnesium, balance substantially aluminum, surrounded by and bonded to an annular body of a magnesium-base alloy containing a substantially higher proportion of magnesium than the core alloy.

In the galvanic consumption of such an anode, the electrolytic potential difference between the alloy of the core and the outer metal is sufficient to maintain the core almost unattacked until the outer metal is virtually all consumed, and yet is not so great that local corrosion of the outer metal is appreciably accelerated when the core is exposed. The occurrence of these desirable effects is further insured by the fact that the core alloy is readily polarizable in the alkaline medium resulting from consumption of the magnesium. However, once the outer metal is entirely consumed, the core itself is still sufficiently anodic to generate an effective though reduced protective current over a significant period.

The invention may be illustrated with reference to the accompanying drawing, in which

2

Fig. 1 is a transverse section through a consumable anode according to the invention; and

Fig. 2 is a diagrammatic vertical section showing the manner of using a consumable anode in the galvanic protection of a buried pipeline.

As stated, the core alloy should contain from about 1 to about 92 percent by weight of magnesium, the balance being substantially aluminum. If the lower limit is passed, the alloy approaches pure aluminum in behavior and is subject to substantial cathodic corrosion and pitting by the alkaline medium produced as the outer core is consumed. If the upper limit is exceeded, the alloy behaves much like magnesium, does not polarize readily, and is not sufficiently cathodic with respect to the outer metal.

In a preferred construction, the core consists of an aluminum-base alloy containing from about 1 to about 12 percent by weight of magnesium as the major alloying element, surrounded by an annular body of a metal containing at least 85 percent magnesium. A typical anode would be one in which the core consists of a commercial aluminum-base alloy containing about 4 percent magnesium, balance substantially aluminum, and the annular body consists of commercially pure magnesium. An anode of this type is illustrated in Fig. 1.

In an alternative construction, the core consists of a magnesium-base alloy containing not over 92 percent by weight of magnesium and the outer body contains more than 95 percent magnesium. For example, a core of a commercial magnesium-base alloy containing 8.5 percent aluminum, 0.5 percent zinc, and 0.2 percent manganese, balance substantially magnesium, is surrounded by a body of commercially pure magnesium.

Anodes of the types described are most conveniently made by a composite extrusion technique. For example, a cylindrical billet of the aluminum-base alloy is inserted in a central bore in a larger cylindrical magnesium billet and the resulting composite billet is forced under heat and pressure through an extrusion die, according to the procedure described in U. S. 2,023,498. In an alternative procedure, the central core is first made by casting and is then centered in a larger mold, and the outer metal cast around it.

A typical installation of an improved anode of the invention is shown in Fig. 2, in which an anode of the type shown in Fig. 1 is used in the galvanic protection of a buried steel pipeline. As illustrated, the anode is buried in a suitably-

sized hole in the earth a short distance from the pipeline and is surrounded by a backfill, such as a bentonite-gypsum mixture, which serves to control the anode environment. An insulated wire electrically connects the core of the anode to the pipeline.

While the new anodes are particularly useful in the protection of underground ferrous metal structures, they may be employed generally in the galvanic protection of ferrous metals immersed in natural aqueous electrolytes, including ground water, fresh water, and seawater. It is necessary only that one or more anodes be immersed in the same body of electrolyte as the structure and be connected electrically to the latter. Typical uses are the protection of ships' bottoms and the prevention of corrosion of domestic hot water heaters. The criteria for choosing the size and number of anodes for a given installation are well known in the art.

It is to be understood that the foregoing description is illustrative rather than limitative, and that the invention is co-extensive in scope with the following claims.

What is claimed is:

1. In combination with a ferrous metal structure immersed in an aqueous electrolyte, galvanic protection means including a consumable anode immersed in the electrolyte and connected electrically to the structure, such anode comprising a core of an alloy containing from about 1 to about 92 per cent by weight of magnesium, balance substantially aluminum, surrounded by and bonded to a body of a magnesium-base alloy containing a substantially higher proportion of magnesium than the core alloy and containing at least 85 per cent magnesium.

2. In combination with a ferrous metal structure immersed in a natural aqueous electrolyte, galvanic protection means including a consumable anode immersed in the electrolyte and connected electrically to the structure, such anode comprising a core of an aluminum-base alloy containing from about 1 to about 12 percent by

weight of magnesium, balance substantially aluminum, surrounded by and bonded to an annular body of a metal containing at least 85 percent magnesium.

3. In combination with a ferrous metal structure immersed in a natural aqueous electrolyte, galvanic protection means including a consumable anode immersed in the electrolyte and connected electrically to the structure, such anode comprising a core of an aluminum-base alloy containing about 4 per cent magnesium, balance substantially aluminum, surrounded by and bonded to an annular body of magnesium.

4. In combination with a ferrous metal structure immersed in a natural aqueous electrolyte, galvanic protection means including a consumable anode immersed in the electrolyte and connected electrically to the structure, such anode comprising a core of a magnesium-base alloy containing not over 92 per cent by weight of magnesium, balance substantially aluminum, surrounded by and bonded to an annular body of a metal containing more than 95 percent magnesium.

JOHN J. GREBE,  
HAROLD A. ROBINSON.

#### REFERENCES CITED

The following references are of record in the file of this patent:

#### UNITED STATES PATENTS

| Number    | Name         | Date          |
|-----------|--------------|---------------|
| 2,011,613 | Brown et al. | Aug. 20, 1935 |
| 2,204,823 | Rhodes       | June 18, 1940 |

#### FOREIGN PATENTS

| Number | Country       | Date |
|--------|---------------|------|
| 2,435  | Great Britain | 1873 |

#### OTHER REFERENCES

"Chemical & Metallurgical Engineering," June 1943, p. 66.

"Corrosion," vol. 1, June 1945, pp. 59 through 69.